

Feb. 27, 1962

E. L. KENT ET AL

3,022,697

ELECTROFORMED MOUTHPIPE AND MOUTHPIECE RECEIVER

Filed Dec. 4, 1956



INVENTORS.  
Earle L. Kent,  
BY David A. LeFevre  
Mueller and Dickel  
Atty's.

1

3,022,697

ELECTROFORMED MOUTHPIPE AND MOUTH-  
PIECE RECEIVEREarle L. Kent and David Albert LeFevre, Elkhart, Ind.,  
assignors to C. G. Conn Ltd., Elkhart, Ind., a corpo-  
ration of Indiana

Filed Dec. 4, 1956, Ser. No. 626,245

2 Claims. (Cl. 84—398)

This invention relates to new and useful improvements in a mouthpipe and mouthpiece receiver for a brass-wind instrument, and more particularly to a one-piece mouthpipe and mouthpiece receiver and method of forming the same.

In brass-wind instruments such as the trumpet, cornet, trombone and the like, the mouthpipe and mouthpiece receiver have previously been formed as separate members. The mouthpipe was usually drawn on a mandrel to obtain the proper inside dimensions. The drawn piece was then cut off at each end to produce the correct inside diameter and length. The mouthpiece receiver was machined by a reaming operation and cut off to give the correct length and inside diameters. The two parts were then assembled by a soldered joint and a sleeve member soldered in a position covering the soldered joint. It has been extremely difficult to maintain closely controlled dimensions at the small end of the mouthpipe and to remove solder from the inside of the mouthpipe-mouthpiece receiver combination when assembled. The dimensions of the mouthpiece receiver and mouthpipe must be maintained to very close tolerances and must be maintained very smooth in order to obtain a part having optimum acoustical properties.

It is therefore one object of this invention to provide a new and improved combined mouthpipe and mouthpiece receiver for a brass-wind instrument having improved acoustical properties.

Another object of this invention is to provide an improved method for preparing a combined mouthpipe-mouthpiece receiver assembly having optimum acoustical properties.

One feature of this invention is the provision of a mouthpipe-mouthpiece receiver combination for a brass-wind instrument which is formed as a single member and has accurately defined interior dimensions and a smooth interior surface having optimum acoustical properties.

Another feature of this invention is the provision of an improved process for preparing one-piece mouthpipe-mouthpiece receiver for a brass-wind instrument by electroforming a layer of metal of desired thickness on a two-piece polished mandrel having dimensions which correspond accurately to the interior of a combined mouthpipe-mouthpiece receiver member having optimum acoustical properties.

Another feature of this invention is the provision of an improved process for preparing a one-piece mouthpipe-mouthpiece receiver combination having a smooth polished interior by electroforming on a two-piece mandrel of desired configuration a thin layer of a corrosion resistant metal, such as nickel, gold, tin, platinum, rhodium, palladium, or corrosion resistant alloys which may be electroplated, followed by electroforming a desired thickness of any desired metal, such as copper or a copper alloy, on the coated mandrel to produce a metal mouthpipe-mouthpiece receiver combination having a smooth plated interior.

In the accompanying drawings, to be taken as part of this specification, there is clearly and fully illustrated a preferred embodiment of this invention, in which drawings,

2

FIG. 1 is a diagrammatic view, partially in section, of an electroplating tank having a mandrel therein for electroforming a mouthpipe-mouthpiece receiver combination.

5 FIG. 2 is a view in section of the plating mandrel with a mouthpipe-mouthpiece receiver combination plated thereon,

FIG. 3 is an exploded view of the plating mandrel and retaining nut therefor shown in FIGS. 1 and 2,

FIG. 4 is a sectional view of the mouthpipe-mouth-  
piece receiver combination with the plating mandrel re-  
moved, and

15 FIG. 5 is a view showing the mouthpipe-mouthpiece receiver combination with the connections to a cornet dotted in to show the relation of this part to its assembly in a typical brass-wind instrument.

This invention consists of an improved one-piece mouth-  
pipe-mouthpiece receiver combination for a brass-wind  
instrument and the method of making the same. In this  
20 invention there is provided a smooth separable plating  
mandrel which tapers outwardly toward each end from  
the point of separation. The mandrel has exterior di-  
mensions which correspond accurately to the interior di-  
25 mensions of a mouthpipe-mouthpiece receiver having  
optimum acoustical properties. The mandrel is electro-  
plated with a thin layer of a protective metal, such as  
nickel, gold, tin, platinum, rhodium, palladium, and then  
30 plated with a thicker layer of any suitable metal, such  
as copper or a copper alloy. When the mandrel is sepa-  
rated and removed from the plated part a hollow tubular  
product is obtained which may be cut to a desired length,  
35 which has a smooth plated interior, of a corrosion re-  
sistant metal, and which is usable as a one-piece mouth-  
pipe-mouthpiece receiver member having optimum acous-  
tical properties.

In FIG. 1 there is shown a plating tank 10 filled with  
a suitable plating liquid 12. A plating electrode 14 is  
40 positioned within the tank 10 adjacent to a plating man-  
drel 16. The electrode 14 and mandrel 16 are connected  
by leads 18 and 20 respectively to a suitable D.C. power  
source such as battery 22.

The plating mandrel 16 is shown in an exploded view  
45 in FIG. 3. The mandrel 16 consists of an elongated  
mandrel part 24, a short mandrel part 36 and a retain-  
ing nut 42. The elongated mandrel part 24 has a very  
slight taper from its smaller end 26 to its enlarged end  
28. The taper of the mandrel part 24 from the end 26  
50 to the enlarged end 28 corresponds very accurately to  
the inner dimensions of a mouthpipe for a brass-wind  
instrument having optimum acoustical properties. The  
enlarged end 28 of the mandrel portion 24 has a threaded  
recess 30 therein for insertion of a tool for removal of  
55 the mandrel part from an electroformed piece. The man-  
drel part 24 has a cylindrical supporting portion 32 ex-  
tending from the smaller end 26 and has a threaded end  
portion 34 for receiving the retaining nut 42. The smaller  
mandrel portion 36 has a substantial taper in the oppo-  
60 site direction from the taper of the mandrel portion 24  
and tapers outwardly on dimensions which define accu-  
rately the inner dimensions of a mouthpiece receiver for  
a brass-wind instrument having optimum acoustical prop-  
erties. When the smaller mandrel portion 36 is fitted on  
65 the elongated mandrel portion 24 the cylindrical portion  
32 extends through the passage 38 in the mandrel portion  
36 with the threads 40 therein partially engaging the  
threads on the cylindrical portion 32. The two mandrel  
portions 36 and 24 are held rigidly together by the nut  
42 which is secured on the threads 34.

The two-part mandrel 16 is placed in the electroform-  
ing bath and plated with a thin continuous layer 44 of  
nickel covering the entire mandrel. The plated mandrel

is then plated with a shell or layer 46 of copper or copper alloy to a selected thickness. The plating mandrel is then removed from the plating bath and the parts of the mandrel separated and withdrawn from the shell 46. The plated shell 46 is a one-piece tubular member having an elongated portion 50 which tapers outwardly toward the end 28 of the plating mandrel. The shell 46 has a smaller portion 48 which tapers outwardly toward the end 34 of the plating mandrel with a much more pronounced taper than the taper of the portion 50. The elongated tapered portion 50 of the shell 46 has internal dimensions which correspond to the exterior dimensions of the plating mandrel and which correspond to a mouthpiece having optimum acoustical properties.

The tapered portion 48 of the shell 46 has dimensions which correspond to the dimensions of the mandrel portion 36 which corresponds to a mouthpiece receiver having optimum acoustical properties. The mouthpiece receiver portion 48 may be cut off as along the dashed line 49 to provide a mouthpiece receiver of suitable length. The nickel layer 44 within the shell 46 provides a smooth continuous layer over the interior of the combined mouthpiece and mouthpiece receiver which is resistant to corrosion, more easily cleaned, and has superior acoustical properties. When removed from the mandrel the shell 46 has accurate internal dimensions but may have an exterior surface which is not so smooth as the interior surface. The exterior of the part may, if desired, be subjected to a machining operation or a chemical stripping operation or a combination of the two to produce the desired external dimensions and surface appearance.

A one-piece mouthpiece-mouthpiece receiver combination which is electroformed in the manner above described has internal dimensions which correspond exactly to the exterior surface of the plating mandrel. A mouthpiece-mouthpiece receiver assembly may be formed more accurately in this manner since there is no spring-back from a plating mandrel as there is from a drawing mandrel. When the part is cut to proper length it may be assembled in a brass-wind instrument such as a trombone, cornet, or trumpet. In FIG. 5 this part is shown assembled in a cornet with a mouthpiece 52 inserted in the mouthpiece receiver portion 48 and with the enlarged end of the mouthpiece 50 inserted into a sleeve 54 which connects to the rest of the cornet assembly 56.

We claim:

1. In a brass-wind musical instrument, a unitary electroformed mouthpiece and mouthpiece receiver adapted to support and position a mouthpiece and form a tone chamber with optimum acoustical properties adjacent the received end of the mouthpiece, said mouthpiece and mouthpiece receiver comprising a one-piece elongated tubular body of seamless and jointless construction including a mouthpiece portion and a mouthpiece receiver portion respectively tapering inwardly from opposite ends of said tubular body to a junction of lesser interior diameter than

either end, said mouthpipe portion being relatively long and having an interior surface of relatively slight taper, and said mouthpiece receiver portion being relatively short and having a frusto-conical interior surface of greater taper than said mouthpiece portion for receiving and accurately positioning the mouthpiece with respect to said junction, said tubular body comprising an interior electroplating of corrosion resistant metal and an exterior electroplating containing at least a major proportion of copper, said platings being continuous and in mutual contact throughout the length of said tubular body, and said interior plating having a highly finished interior surface of accurate circular cross-section having a diameter at any portion thereof which has a predetermined value with minimum tolerance variation so that the spacing between the received end of the mouthpiece and said junction has a predetermined value with minimum tolerance variation.

2. In a brass-wind musical instrument, a unitary electroformed mouthpipe and mouthpiece receiver adapted to support and position a mouthpiece and form a tone chamber with optimum acoustical properties adjacent the received end of the mouthpiece, said mouthpipe and mouthpiece receiver comprising a one-piece elongated tubular body of seamless and jointless construction including a mouthpipe portion and a mouthpiece receiver portion respectively tapering inwardly from opposite ends of said tubular body and joined at the smaller ends thereof, said mouthpipe portion being relatively long and having an interior surface of relatively slight taper, and said mouthpiece receiver portion being relatively short and having a frusto-conical interior surface of greater taper than said mouthpipe portion for receiving and accurately positioning the mouthpiece therein, said tubular body comprising an interior electroplating of corrosion resistant metal and an exterior electroplating of metal substantially thicker than said interior electroplating and providing substantial strength to the tubular body, said platings being continuous and in mutual contact throughout the length of said tubular body, and said interior plating having a highly finished interior surface of accurate circular cross-section and having a diameter at any portion thereof which has an accurately predetermined value.

45

#### References Cited in the file of this patent

#### UNITED STATES PATENTS

|           |            |                |
|-----------|------------|----------------|
| 1,178,330 | Mackey     | Apr. 4, 1916   |
| 1,385,202 | Couturier  | July 19, 1921  |
| 1,509,104 | Hickernell | Sept. 23, 1924 |
| 1,694,962 | Berry      | Dec. 11, 1928  |
| 2,613,178 | Grant      | Oct. 7, 1952   |

#### FOREIGN PATENTS

|    |         |         |               |
|----|---------|---------|---------------|
| 55 | 115,494 | Germany | Dec. 12, 1900 |
|    | 378,157 | France  | Aug. 1, 1907  |